

## 1

3,424,680

## SOIL RETARDANT COMPOSITIONS AND TEXTILE MATERIALS

William Julius van Loo, Jr., Middlesex, and George Robert De Paolo, Whitehouse Station, N.J., assignors to American Cyanamid Company, Stamford, Conn., a corporation of Maine  
 No Drawing. Filed Aug. 5, 1965, Ser. No. 477,575  
 U.S. Cl. 252—8.8 19 Claims  
 Int. Cl. D06m 13/40

### ABSTRACT OF THE DISCLOSURE

Compositions effective for imparting soil retardance to textiles which comprise a compound of the formula



wherein R is selected from the group consisting of alkyl, alkenyl and alkadienyl having from about 12 to 22 carbon atoms, said compound being dispersed in an alcoholic solution or in an aqueous solution with an imidazolinium compound such as N-(2,3-dihydroxypropyl)-N-(2-hydroxyethyl)-2-heptadecylimidazolinium chloride. The invention also includes a method of imparting soil retardance to carpets by application of the composition and carpet fabrics having thereon the dry residue of the composition.

This invention relates to compositions useful for imparting soil retardance to textile materials, to methods of rendering textile materials soil retardant and to the resultant soil retardant textiles.

More particularly, the invention pertains to compositions and methods effective for improving the resistance to soiling or for reducing the adherence or attraction of soil particles to textile materials such as flat or pile carpets.

Currently, in the rug and carpet industry, widespread use is being made of fibers other than wool in making carpet pile. Additionally, the carpets thus made are being offered in light or pastel colors. Such developments have given rise to an increased need for effective and long-lasting soil retardants to justify the costly installation of such carpets, which are more readily soiled than wool carpets and, when light colored, more readily exhibit soiling.

Soil retardants heretofore used or suggested include colloidal dispersions of inorganic oxides, such as silica, alumina, titania, and the like. These inorganic colloids are useful to some degree but have short service life, especially when carpets treated therewith are vacuumed. The inorganic colloids also cause discoloration or whitening of the treated carpets so that an undesirable change in shade occurs even before the carpet is put into service use.

Certain other soil retardants of organic nature have been employed. This type also suffers from deficiencies including one or more of the following, depending on the specific organic variety: (1) not universally effective on carpets of all fiber types; (2) impart stiffness or rigidity to the carpet pile resulting in undesirable "hand" or lie of such pile and embrittlement thereof; (3) cause discoloration or whitening of the carpet leading to an undesirable change in shade even before service use; (4) lack reasonable durability to service use and cleaning, particularly when vacuuming; (5) require uneconomical usage levels for effectiveness. There exists, therefore, a continuing and increasing need for soil retardants which are effective on carpets of all fiber types and which overcome the deficiencies of the prior art soil retardants.

An object of the invention is to provide compositions

## 2

of matter useful for imparting durable soil resistance or retardance to textile materials, particularly flat or pile carpets of all types, without causing discoloration or rigidity.

Another object of the invention is to provide a method for imparting durable soil retardance to textile materials such as flat or pile carpets.

A further object of the invention is to provide soil retardant textiles, particularly carpets of all fiber types and color, which also substantially retain their original coloration and "hand," even after repeated vacuumings.

These and other objects, features and advantages of the invention are further detailed in the description which follows.

15 The foregoing objects are accomplished by treating textile materials with compounds of the formula



The compounds of Formula I are conveniently prepared by reacting ammonia with the appropriate glycidyl ester as follows wherein R is as already defined:



Further details of this process are disclosed in U.S. application Ser. No. 425,627, filed Jan. 14, 1965, which is incorporated herein by reference.

Compounds of this class useful for imparting soil retardance include:



as well as mixtures thereof, e.g., amides prepared from coconut oil acid mixtures.

Compounds of Formula I may be applied to fibrous materials as alcoholic solutions, alcohol-water solutions, or as aqueous dispersions employing imidazolinium compounds as dispersants, with or without a water-soluble alcohol.

45 When the compounds of Formula I are applied from alcoholic solutions, suitable alcohols include water-soluble or substantially water-insoluble alcohols. Effective water-insoluble alcohols are methanol, ethanol, propanol, isopropanol, and the like, and effective substantially water-insoluble alcohols include tertiary butanol, hexanol, and the like. Sufficient alcohol or alcohol-water mixture should be employed to dissolve or disperse the amide. Generally, in alcohol-water mixtures, the alcohol should comprise at least 25% by weight of solvent.

55 The imidazolinium dispersants are quaternary cationic imidazolinium salts of the formula



wherein R<sup>1</sup> is higher alkyl, i.e., having at least 8 carbon atoms and preferably from 12 to 22 carbon atoms; R<sup>2</sup> and R<sup>3</sup> are each selected from the group consisting of hydroxy- and polyhydroxy-substituted alkyl; and X<sup>-</sup> is an anion, preferably halogen but also including NO<sub>3</sub><sup>-</sup>, SO<sub>4</sub><sup>2-</sup>, H<sub>2</sub>SO<sub>4</sub><sup>-</sup>, methosulfates, e.g., CH<sub>3</sub>OSO<sub>3</sub><sup>-</sup>, and the like. R<sup>2</sup> and R<sup>3</sup> may be the same or different and preferably contain 1 to 7 carbon atoms, i.e., lower alkyl. A particularly effective cationic imidazolinium dispersant is N-(2,3-dihydroxypropyl)-N-(2-hydroxyethyl)-2-heptadecylimidazolinium chloride.

The amide and imidazolinium dispersant may be employed in an amide:dispersant ratio of from 2:1 to 35:1, preferably 3:1 to 25:1, together with sufficient water or water-alcohol mixture for the desired fluidity. When the treated textile material is to be used under moist or humid conditions, as during humid summer months, less dispersant is desirable. A preferred range under these conditions is 24:1 to 30:1, same basis.

The compounds may effectively be applied to materials containing fibers of all types, natural and synthetic, singly or as blends. Such fibers include cotton, rayon, wool, nylon, acrylics, polyesters, and the like. Preferably, the fibers are in the form of a carpet with loop or cut pile. Such carpets may contain a backing material of known composition and, additionally, may have whatever backing treatment is appropriate. For example, the backing material may be jute (burlap), alone or impregnated with known resins, and may be further supported with nonslip foam rubber. Flat or hooked carpets are also made soil retardant in accordance with the invention.

The treating compositions are applied to finished fibrous textile materials or during manufacture thereof any suitable means such as dipping, padding, spraying, coating, and the like. For application to carpets, spraying is the preferred technique, although mechanical applicators may be used on previously installed carpeting. The amount of solids of the composition applied to the fibrous material is not critical and may vary from about 0.1 to about 10.0% based on the weight of the fibrous material. Preferably, the amount of solids applied to carpet pile will be between 0.25 and 5.0% based on the weight of said pile. The treating composition should contain sufficient solids to deposit the required amount on the fibrous material by the particular application method employed.

After the treating composition has been applied, the fibrous material is allowed to dry so as to remove the alcohol and/or water. Drying may be accomplished at ambient conditions or, where possible, at elevated temperatures. The use of ovens circulating hot air at about 140° F. has been found particularly advantageous. The time required for drying in such ovens is about four hours.

The amides of Formula I are useable as crude reaction mixtures directly from the reaction medium from which they are prepared, thus avoiding the expense of additional processing, although purified products may be used, if desired.

Moreover, the amides alone, or in admixture with the imidazolinium dispersants, may be transported as a dry powder and thereafter, at place of use, dissolved or dispersed as described to form the treating compositions.

The effective soil retardance imparted by the combination of amide and imidazolinium salt is an unexpected and surprising result in view of the fact that compositions containing imidazolinium salts are known to have the opposite effect, i.e., impart soil retaining or scavenging properties to textiles, which properties improve in alcoholic solution. See U.S. Patent 3,105,500. This is further evidence of the unpredictability of result when known dispersants and other compounds are applied to fabrics such as carpets. The result is surprising also since, as demonstrated hereinafter, the use of anionic, nonionic and other cationic dispersants in combination with amides of Formula I, was unsuccessful and in some cases (cationics) produced an opposite effect, i.e., soil retention.

While the invention is not to be limited by any theory of operation, it is believed that the superior soil retardance observed when cut or loop pile carpets are treated according to the invention is due to filling in of the interstices and cavities of such fibers by the treating compounds. These fiber interstices, in the absence of treatment, appear to attract and hold soil particles which are then difficult to displace by vacuuming. By filling in such cavities, a relatively smooth surface results from which soil may be more readily removed.

When treated with the amides from alcoholic or alcohol-water dispersions according to the invention, carpets and rugs also exhibit water repellency and particularly resistance to soiling by beverages such as tomato juice, grape juice, cola and the like. This property is also observed when the treating compositions contain the imidazolinium salts, although to a lesser extent.

To further illustrate the invention, the following examples are given in which all parts and percentages are by weight unless otherwise specified. Any specific enumeration of detail contained therein should not be interpreted as a limitation on the case except where indicated in the appended claims.

#### EXAMPLE 1

An aqueous ethanol solution (2:1 H<sub>2</sub>O:ethanol) containing 2% solids of N-(2,3-dihydroxypropyl)stearamide was applied by spraying to a 12" x 12" carpet sample consisting of 50% cut nylon pile and 50% burlap backing. Spraying was confined to the pile and the carpet sample increased 50% in weight. Since the carpet increased in weight by 50% and contained 50% pile to which the spray was directed, it may be concluded that the pile actually increased in weight by 100% and thus the pile contained compound solids equal to the concentration in the application bath, that is, 2%. The treated carpet was dried in an oven circulating hot air at 60° C. After drying, the carpet was vacuumed to remove loose pile and incidental dirt.

Soiling tests were then conducted by placing the treated carpet along with untreated carpets on the floor in a special pattern. The carpets were exposed to traffic, e.g., dry soil, wet soil, tarry deposits, and the like. The design of the samples was changed periodically according to a plan similar to that proposed by the American Association of Textile Chemists and Colorists (A.A.T.C.C.), American Dyestuff Reporter, May 13, 1963, pages 56-93. After each pattern change, the A.A.T.C.C. recommendations were followed to a predetermined level of soiling and included vacuuming. Reflectance measurements were made on the carpets before and after exposure to soiling, and soil index values calculated as described in "Accelerated Soiling Test—Juvenon Soil Retardant R," Textile Finishing Bulletin No. 148A, American Cyanamid Co., Bound Brook, N.J., December 1955. Results of the tests on the above treatment are shown in Table I. The percent weights of treating agent in this and succeeding examples are based on the weight of pile in the carpet samples.

Table I.—Service soiling of nylon carpets

| Treatment:                           | Soil index |
|--------------------------------------|------------|
| None                                 | 1.00       |
| 2% N-(2,3-dihydroxypropyl)stearamide | 0.52       |

Values of soil index below 1.00 indicate soil retardancy; hence, the lower the value the more favorable is the soil retardancy. Good soil retardants generally have soil indices below about 0.70. When a soil index value is greater than 1.00 it indicates that soil retention or scavenging is being effected. The untreated control in a service soiling test is arbitrarily assigned a soil index of 1.00 and performance of other samples are calculated on such basis.

The results of this experiment show the desirable soil retardancy obtained with a compound of the present invention when application is made from an aqueous alcohol solution.

#### EXAMPLE 2

Following the procedure of Example 1, N-(2,3-dihydroxypropyl)stearamide was again applied to a nylon carpet sample and to another carpet sample a N-(2,3-dihydroxypropyl)amide derived from distilled coconut oil

fatty acids was similarly applied. The acid content of such coconut oil is typically as follows:

| Acid     | Formula                                                                                         | Content |
|----------|-------------------------------------------------------------------------------------------------|---------|
| Caprylic | $\text{CH}_3(\text{CH}_2)_8\text{COOH}$                                                         | 8       |
| Capric   | $\text{CH}_3(\text{CH}_2)_10\text{COOH}$                                                        | 7       |
| Lauric   | $\text{CH}_3(\text{CH}_2)_12\text{COOH}$                                                        | 48      |
| Myristic | $\text{CH}_3(\text{CH}_2)_14\text{COOH}$                                                        | 18      |
| Palmitic | $\text{CH}_3(\text{CH}_2)_16\text{COOH}$                                                        | 9       |
| Stearic  | $\text{CH}_3(\text{CH}_2)_18\text{COOH}$                                                        | 2       |
| Oleic    | $\text{CH}_3(\text{CH}_2)_17\text{CH}=\text{CH}(\text{CH}_2)\text{COOH}$                        | 8       |
| Linoleic | $\text{CH}_3(\text{CH}_2)_17\text{CH}=\text{CHCH}_2\text{CH}=\text{CH}(\text{CH}_2)\text{COOH}$ | 1       |

The treated carpets were tested in the manner of Example 1 with results as follows:

Table II.—Service soiling of nylon carpets

| Treatment:                             | Soiling index |
|----------------------------------------|---------------|
| None                                   | 1.00          |
| 2% N-(2,3-dihydroxypropyl)stearamide   | 0.66          |
| 2% N-(2,3-dihydroxypropyl)coconutamide | 0.69          |

These results show that desirable soil retardancy is obtained with treating agents of differing amide carbon content. It will be noted that the soil index value obtained with N-(2,3-dihydroxypropyl)stearamide is somewhat higher in Example 2 than in Example 1. This is a normal variation expected in separate service soiling tests since the nature and type of soil encountered in the separate exposures of Examples 1 and 2 obviously cannot be controlled. However, the relative effectiveness in Example 2 of the amides of different carbon chains is clear since they were evaluated at the same time.

## EXAMPLE 3

Aqueous alcohol solutions of different solids contents of N-(2,3-dihydroxypropyl)stearamide were applied to nylon carpet samples as in Example 1 so as to deposit 0.5, 1.0, 2.0, and 3.0% solids of N-(2,3-dihydroxypropyl)stearamide based on the weight of the carpet pile. Accelerated soiling tests as in Examples 1 and 2 were run on the treated samples. Results are given in Table III and show increasing soil retardancy with increasing applied solids.

Table III.—Accelerated solids of nylon carpets

| Concentration of N-(2,3-dihydroxypropyl)stearamide (percent solids): | Soil index |
|----------------------------------------------------------------------|------------|
| None                                                                 | 1.00       |
| 0.5                                                                  | 0.77       |
| 1.0                                                                  | 0.72       |
| 2.0                                                                  | 0.62       |
| 3.0                                                                  | 0.59       |

## EXAMPLE 4

Aqueous dispersions of the following compositions were applied to the same carpet type described in Example 1 using the same procedure as therein described. The compositions contained N-(2,3-dihydroxypropyl)stearamide (NDHPSA) and various dispersants as follows wherein the numbers are parts by weight:

## DISPERSANT COMPOSITIONS

|                         | A    | B    | C    | D    | E    | F    |
|-------------------------|------|------|------|------|------|------|
| NDHPSA                  | 1.72 | 1.72 | 1.72 | 1.72 | 1.72 | 1.72 |
| D-1                     | .27  |      |      |      |      |      |
| D-2                     |      | .28  |      |      |      |      |
| D-3                     |      |      | .28  |      |      |      |
| D-4                     |      |      |      | .28  |      |      |
| D-5                     |      |      |      |      | .28  |      |
| D-6                     |      |      |      |      |      | .28  |
| $\text{H}_2\text{O}$ to | 100  | 100  | 100  | 100  | 100  | 100  |

The dispersants are identified as follows:

- D-1—N-(2,3-dihydroxypropyl)-N-(2-hydroxyethyl)-heptadecyl imidazolinium chloride
- D-2—Lauramidopropylidemethyl-beta-hydroxyethylammonium methosulfate
- D-3—Stearamidopropyl dimethyl-beta-hydroxyethylammonium nitrate
- D-4—Potassium toluenesulfonate
- D-5—Nonyl phenol-ethylene oxide adduct, 1:9 mole ratio, respectively.
- D-6—Octadecyl trimethylammonium chloride

Soiling tests were run as in Example 1 with the results shown in Table IV.

Table IV.—Service soiling of nylon carpets

|    | Dispersant composition: | Soil index |
|----|-------------------------|------------|
| 5  | None                    | 1.00       |
|    | A                       | 0.49       |
|    | B                       | 2.22       |
|    | C                       | 1.30       |
|    | D                       | 1.15       |
| 10 | E                       | 1.04       |
|    | F                       | 1.57       |

The carpet samples treated with compositions B, C and F were removed from the test pattern after five days because of heavy soiling and possibility of contamination of other samples by soil transfer. The soil indices represent comparative soiling of these samples relative to the untreated sample exposed to the full 16-day soiling test. These soil indices, in effect, would be considerably greater if the samples were exposed for the full test duration or were compared to untreated carpets exposed for only five days.

These results show the specificity of dispersants useful in the present invention. Specificity is not only restricted to the cationic class but also to a particular species within a class. The results also show that aqueous dispersions of the proper composition are effective in producing desirable soil retardancy.

## EXAMPLE 5

Example 1 was repeated except that additional, separate applications were made to carpets of similar construction containing cut pile of the various types listed in Table V with results as shown therein. Testing was as in Example 1.

Table V.—Service soiling of various carpets

| Pile fiber:           | Soil index |
|-----------------------|------------|
| Nylon                 | 0.51       |
| Wool                  | 0.35       |
| Viscose               | 0.65       |
| Orlon acrylic fiber   | 0.42       |
| Creslan acrylic fiber | 0.38       |

The soil index values are relative to an untreated control carpet of same type having an assigned soil index of 1.00 and exposed to soiling at the same time.

This example shows that the compositions of the present invention are useful in imparting soil retardancy to carpets having pile of various fiber types.

## EXAMPLE 6

Colloidal aqueous dispersions of alumina, silica, and titania were applied to nylon carpets according to the procedure of Example 1, except that the carpets were dyed in medium green shade. NDHPSA [N-(2,3-dihydroxypropyl)stearamide] was also applied to another sample of the same carpet material according to Example 1. A copolymer of sodium vinyl sulfonate and acrylamide was similarly applied to still another sample of the same material.

Following treatment and drying, the carpets were examined visually for effect on shade and manually for effect on pile suppleness. The carpets treated with alumina and titania whitened considerably as a result of treatment while that treated with silica yellowed to a considerable extent. The other treated carpets were unchanged in shade from the untreated.

The pile of the carpet treated with the copolymer was very firm and rigid as a result of treatment and the pile of the carpets treated with the inorganic colloids was slightly firm. However, the pile of the carpet treated with NDHPSA remained as soft and supple as untreated samples.

The carpets were subjected to soiling tests as in Example 1 except that visual ratings of the soilings were made instead of reflectances because of the color problem oc-

casioned by the dye. All the carpet samples exhibited good soil retardancy after the few days of exposure. However, as exposure increased and as the samples were vacuumed, performance of the inorganic colloids and the copolymer became inferior to that of NDHPSA. After the full cycle of exposure to soiling and vacuuming, only the carpet treated with NDHPSA showed a clear advantage over the untreated carpet, i.e., a definitely cleaner, lighter shade, thus demonstrating the superiority of the treating agents of the present invention over known soil retardants.

We claim:

1. A composition of matter effective for imparting soil retardance to textiles which consists essentially of an alcoholic solution of an amide of the formula



wherein R is selected from the group consisting of alkyl, alkenyl and alkadienyl having from about 12 to 22 carbon atoms the alcohol being a monohydric aliphatic alcohol of 1 to 6 carbon atoms and constituting at least 25 percent by weight of the solvent medium of said solution.

2. A composition of matter as in claim 1 wherein said solution also contains water.

3. A composition of matter effective for imparting soil retardance to textiles which consists essentially of a dispersion of from 2 to 35 parts by weight of an amide of the formula



wherein R is selected from the group consisting of alkyl, alkenyl and alkadienyl having from about 12 to 22 carbon atoms in an aqueous solution of one part of an imidazolinium compound of the formula



wherein R<sup>1</sup> is higher alkyl; R<sup>2</sup> and R<sup>3</sup> are each selected from the group consisting of hydroxy- and polyhydroxy-substituted lower alkyl; and X<sup>-</sup> is an anion.

4. A composition of matter as in claim 1 wherein said amide is N-(2,3-dihydroxypropyl)coconutamide.

5. A composition as in claim 1 wherein said amide is N-(2,3-dihydroxypropyl)stearamide.

6. A composition as in claim 3 wherein said amide is N-(2,3-dihydroxypropyl)stearamide and said imidazolinium compound is N-(2,3-dihydroxypropyl)-N-(2-hydroxyethyl)-2-heptadecylimidazolinium chloride.

7. A composition as in claim 3 wherein said amide is N-(2,3-dihydroxypropyl)stearamide and said imidazolinium compound is N-(2,3-dihydroxypropyl)-N-(2-hydroxyethyl)-2-heptadecylimidazolinium chloride.

8. A method of imparting soil retardancy to carpets which comprises applying thereto an effective amount of an amide of the formula



wherein R is selected from the group consisting of alkyl, alkenyl and alkadienyl having from about 12 to 22 carbon atoms.

9. A method as in claim 8 wherein said amide is N-(2,3-dihydroxypropyl)stearamide.

10. A method as in claim 8 wherein said amide is N-(2,3-dihydroxypropyl)coconutamide.

11. A method as in claim 8 wherein said amide is applied from an aqueous solution containing a monohydric alcohol of about 1 to 6 carbon atoms.

12. A method as in claim 11 wherein the alcohol is ethanol.

13. A method of imparting soil retardancy to carpets

which comprises applying an effective amount of an aqueous solution of an amide of the formula



- 5 where R is selected from the group consisting of alkyl, alkenyl and alkadienyl having from about 12 to 22 carbon atoms, said solution also containing a dispersant amount within the range of one part for each 2 to 35 parts by weight of said amide of an imidazolinium compound of the formula



wherein R<sup>1</sup> is higher alkyl; R<sup>2</sup> and R<sup>3</sup> are each selected from the group consisting of hydroxy- and polyhydroxy-substituted lower alkyl; and X<sup>-</sup> is an anion.

- 20 14. Carpet fabric having thereon the dry residue of a solution in a volatile alcoholic solvent of an amide of the formula



25 wherein R is selected from the group consisting of alkyl, alkenyl and alkadienyl having from 12 to 22 carbon atoms, wherein the amount of said residue is effective to impart soil retardance to said carpet fabric.

- 30 15. Carpet fabric as in claim 14 wherein said amide is N-(2,3-dihydroxypropyl)coconutamide.

16. Carpet fabric as in claim 14 wherein said amide is N-(2,3-dihydroxypropyl)stearamide.

- 35 17. Carpet fabric having thereon the dry residue of an aqueous solution of an amide of the formula



40 wherein R is selected from the group consisting of alkyl, alkenyl and alkadienyl having from about 12 to 22 carbon atoms, said aqueous solution containing a dispersant amount within the range of one part for each 2 to 35 parts by weight of said amide of an imidazolinium compound of the formula



wherein R<sup>1</sup> is higher alkyl; R<sup>2</sup> and R<sup>3</sup> are each selected from the group consisting of hydroxy- and polyhydroxy-substituted lower alkyl; and X<sup>-</sup> is an anion, wherein the amount of said residue is effective to impart soil retardance to said carpet fabric.

- 45 18. Carpet fabric as in claim 17 wherein said amide is N-(2,3-dihydroxypropyl)stearamide and said imidazolinium compound is N-(2,3-dihydroxypropyl)-N-(2-hydroxyethyl)-2-heptadecylimidazolinium chloride.

- 50 19. Carpet fabric as in claim 17 wherein said amide is N-(2,3-dihydroxypropyl)stearamide and said imidazolinium compound is N-(2,3-dihydroxypropyl)-N-(2-hydroxyethyl)-2-heptadecylimidazolinium chloride.

#### References Cited

#### UNITED STATES PATENTS

|           |         |                |         |
|-----------|---------|----------------|---------|
| 2,002,613 | 5/1935  | Orthner et al. | 260—404 |
| 2,876,140 | 3/1959  | Sheehan        | 252—8.8 |
| 2,957,003 | 10/1966 | Johnson        | 252—8.8 |

HERBERT B. GUYNN, Primary Examiner.

U.S. CL. X.R.